

March 31, 1970

T. EDSTROM

**3,504,065**

METHOD FOR SUPPRESSING THE ESCAPE OF VOLATILES WHILE  
PRESSURE BAKING CARBON ARTICLES  
Original Filed Aug. 15, 1966

Original Filed Aug. 15, 1966

FIG. I



FIG. 2



**INVENTOR.**  
**THEODORE EDSTROM**

BY *John C. G.*

*Robert L. Clegg*  
**ATTORNEY**

1

3,504,065

## METHOD FOR SUPPRESSING THE ESCAPE OF VOLATILES WHILE PRESSURE BAKING CARBON ARTICLES

Theodore Edstrom, Parkview, Ohio, assignor to Union Carbide Corporation, a corporation of New York  
Continuation of application Ser. No. 572,573, Aug. 15, 1966. This application May 1, 1969, Ser. No. 824,361  
Int. Cl. B29c 25/00; C01b 31/00  
U.S. Cl. 264—29

3 Claims

### ABSTRACT OF THE DISCLOSURE

An improved method for making a formed carbon article is provided. The method includes the simultaneous application of a mechanical and pneumatic pressure while heating a carbonaceous charge to a carbonization temperature. The charge is initially provided with a high binder content which together with the use of a pneumatic pressure which suppresses the escape of volatiles from the charge enables a strong, highly dense article to be produced.

This application is a continuation of Ser. No. 573,573 filed Aug. 15, 1966, now abandoned.

This invention relates to the production of carbon and graphite masses and more particularly to an improved process of pressure baking carbon articles.

A recently developed pressure baking method for producing carbon articles comprises confining, in a refractory lined mold, a mixture of finely divided carbonaceous particles with a fusible and carbonizable carbonaceous binder susceptible of thermal decomposition, subjecting the mixture within the mold to a high mechanical pressure of the order of 4500 pounds per square inch to compress the same, and passing an electrical current of about 500 amperes per square inch of compressed mixture in the mold to heat the mixture to a temperature at which substantially complete carbonizing of the binder constituent occurs. By means of this process, it is possible to produce in about eight minutes carbon articles which heretofore required a production time of eight weeks.

In the above-described process, pitch and certain other binder materials produce volatile substances which condense on the press, punches, and cold sections of the mold. Accumulation of such substances prevents or interferes with proper operation of the equipment, and in an extreme case can occasion minor explosions.

A recent improvement in the above described process which overcomes this particular disadvantage and which enables the use of higher binder concentrations is disclosed in U.S. Patent 2,965,931 wherein it is shown that the evolution of condensable hydrocarbons can be substantially eliminated by adding finely divided sulfur to the mix blend to react with the pitch component, thereby causing the evolved gas to become non-condensable and yielding a higher percentage deposition of bonding coke. However, in addition to the fact that sulfur in the pitch bonded mix creates gases which are toxic and which are corrosive, the use of sulfur in certain carbon products is sometimes undesirable because the operating properties of the product are affected. For example, in the manufacture of carbon brushes the presence of a bond resulting from coke which has been deposited in the presence of sulfur causes relatively high friction during commutation.

The principal object of this invention therefore, is to provide a method of pressure baking carbon articles whereby the evolution of condensable hydrocarbons is substantially eliminated without the use of a sulfur additive.

Another primary object of this invention is to provide a method of pressure baking carbon articles whereby higher

2

binder concentrations may be employed without the use of a sulfur additive.

These and other objects of this invention will become apparent from the following description, taken in conjunction with the accompanying drawing wherein

FIGURE 1 is an apparatus which may be suitably employed in the process of the invention; and

FIGURE 2 is a schematic of an auxiliary pressure supply and control system.

Broadly stated, the objects of the invention are accomplished by the application of a pneumatic pressure to a carbonaceous charge while the charge is being subjected to heat and mechanical pressure. The pneumatic pressure is preferably applied by contacting the charge with a gas in a sealed chamber. The gas suppresses the escape of hydrocarbon volatiles from the charge with the result that the hydrocarbons are retained in a liquid phase and are forced to coke during the carbonization process. Thus the presence of condensates on the pressing ram and other equipment is eliminated. Furthermore, a greater carbon yield is achieved and higher binder concentrations may be employed.

Any gas may be employed in the instant process which does not oxidize the carbonaceous mix. Such gases include nitrogen, argon, helium, carbon monoxide and the like.

The pneumatic pressure is preferably applied prior to the application of the mechanical pressure and then maintained thereafter. Furthermore, it may be increased or decreased during operation as will be hereinafter further described. For best results, a pneumatic pressure of at least 10 p.s.i. and as high as 2000 p.s.i. or greater is applied while a mechanical pressure of about 500 to 4000 p.s.i. compresses the carbonaceous charge. A pneumatic pressure of between 50 p.s.i. and 1000 p.s.i. is preferred.

Referring to FIGURE 1, an apparatus 10 suitable for use in the process of the invention comprises a steel cylinder 12 which encloses a high temperature ceramic liner 14 and a carbon liner 16. Adjacent the carbon liner 16 is a graphite mold 18. A carbonaceous charge 20 having been surrounded by coke packing 22, is situated within the area defined by the graphite mold 18. Mechanical pressure is applied through a graphite ram 24 which may also serve as an electrical conductor to supply current to the charge 20. The apparatus is sealed by means of Teflon<sup>1</sup> gasket 26 and asbestos seal ring 28 thereby preventing the escape of volatiles or gas. A gas inlet conduit 30 passes through a steel cover 32 and contacts the chamber 34 by means of a passage 35 around the ram extension 36 and the graphite ram 24.

In operation, a non-oxidizing gas is fed into the chamber 34 through the gas inlet conduit 30 by placing a gas feeding means at the opening 31 of the conduit. A pneumatic pressure is thereby applied to the carbonaceous charge 20 and escape of hydrocarbon volatiles from the charge is prevented. Mechanical pressure is applied to charge through the ram 24 while the charge is baked. Upon completion of the process, the graphite ram is withdrawn and the non-oxidizing gas is permitted to escape through inlet conduit 30 by means of valve 46 as illustrated in FIGURE 2.

It will be appreciated that the pneumatic pressure which is applied to the charge will be dependent on the volume of the chamber 34, the quantity of gas which is fed into the chamber, and the temperature to which the gas is subjected. Normal expansion of the gas during heating will, of course, increase the pneumatic pressure since the apparatus is completely sealed. However, the pressure may be maintained at a desired value by releasing gas from the system during the process. This may be readily accomplished by one skilled in the art through the use of

<sup>1</sup> Teflon—registered trademark of Du Pont Corporation—a plastic consisting of a tetrafluoroethylene polymer.

valves and the like which could conveniently be attached to the system as illustrated in FIGURE 2.

Referring now to FIGURE 2, a typical pressure supply and control system comprises a gas containing means 38, a compressor 40 which places the gas under pressure, a pressure regulated by-pass valve 42 connected across the compressor 40, a pressure inlet valve 44, a pressure re-

M.P.). One group of samples contained 10 parts of binder per hundred parts of coke flour and another group contained 20 parts per hundred. The accompanying Table I shows the baked density, strength, and resistivity of these samples compared to control samples (Tests No. 1 and No. 4) which were not prepared under pneumatic pressure.

TABLE I

| Test No. | Pitch Cone., p.p.h. | Power input, kw. | Time on fire, sec. | Estimated final temp., °C. | Gas Pressure (p.s.i.) | Apparent density, gm./cc. | Resistivity, ohm-inch | Flexural strength, p.s.i. | Applied mech. pressure, p.s.i. | Effective mech. pressure, p.s.i. |
|----------|---------------------|------------------|--------------------|----------------------------|-----------------------|---------------------------|-----------------------|---------------------------|--------------------------------|----------------------------------|
|          |                     |                  |                    |                            | Initial Maximum       |                           |                       |                           |                                |                                  |
| 1-----   | 10                  | 66               | 45                 | 1,200                      | 1 0 0                 | 1.565                     | 0.00299               | 1,210                     | 4,000                          | 4,000                            |
| 2-----   | 10                  | 73               | 52                 | 1,400                      | 0 500                 | 1.569                     | 0.00242               | 1,650                     | 4,000                          | 4,000-3,500                      |
| 3-----   | 10                  | 55               | 46                 | 1,000                      | 600 1,000             | 1.576                     | 0.00224               | 1,880                     | 4,000                          | 3,400-3,000                      |
| 4-----   | 20                  | 65               | 36                 | 1,100                      | 0 0                   | 1.49                      | 0.00654               | 2,170                     | 4,600                          | 4,600                            |
| 5-----   | 20                  | 66               | 35                 | 1,100                      | 0 1,000               | 1.649                     | 0.00250               | 2,390                     | 4,600                          | 4,600-3,600                      |
| 6-----   | 20                  | 70               | 81                 | 1,250                      | 600 1,650             | 1.652                     | 0.00240               | 2,650                     | 4,600                          | 4,000-2,350                      |
| 7-----   | 20                  | 66               | 46                 | 1,100                      | 1,000 1,500           | 1.629                     | 0.00250               | 2,620                     | 4,600                          | 3,600-3,100                      |

<sup>1</sup> 0 denotes atmospheric pressure. <sup>2</sup> Applied mechanical pressure less pneumatic pressure.

lease valve 46 to insure safety and to control the pressure applied, pressure gauge 48 which measures the pneumatic pressure at all times and gauges 50, 52 which measure container pressure and line pressure: In operation this system is able to closely regulate the pneumatic pressure to be applied to the charge by controlling the quantity of gas, such as nitrogen which is supplied to the chamber 34.

Although a pressure supply and control system such as that illustrated in FIGURE 2 is the preferred equipment for applying a pneumatic pressure, any manner of application is within the concept of the invention. For example, a pneumatic pressure may be applied to the charge without the use of an external gas by simply sealing the apparatus as hereinbefore illustrated. During heating, volatiles will escape from the charge but not from the chamber 34. Since the escape of the volatiles from the apparatus is prevented, a pneumatic pressure is formed in the chamber as the volatiles continue to egress from the charge. At some point in the process, equilibrium will be accomplished and no further escape of volatiles from the charge will occur due to the pressure in the chamber. In this manner, pneumatic pressure is applied to the charge without the use of an external nonoxidizing gas. It will be appreciated that control of the pneumatic pressure is less precise than that achieved with the use of an external gas and in addition, some volatilization will occur. However, by decreasing the size of the chamber 34, equilibrium is realized in a relatively short time, and the process is quite effective since the escape of volatiles from the charge is still substantially suppressed. Control may be realized by connecting an escape valve such as that illustrated by the numeral 46 in FIGURE 2.

A number of tests evaluating the effectiveness of the invention were performed and are set forth below. Each of the tests was performed with apparatus and equipment similar to that illustrated in the drawing.

#### EXAMPLE I

A series of 2" diameter by 2½" long cylindrical

Table I indicates that at the lower pitch concentration, used in tests 1, 2, and 3, which is representative of a level near the maximum effectively employable without the application of pneumatic pressure, an increase in flexural strength and reduction in electrical resistivity resulted with an application of a pneumatic pressure. At the higher binder level, the end product made without pneumatic pressure (test 4) displays an even lower apparent density, and the specific electrical resistance is even higher, than the product made at 10 p.p.h. The marked improvement in density and flexural strength as well as the lower resistivity obtained with the application of pneumatic pressure at the higher binder concentration is evident from a comparison of test 4 results with those obtained from tests 5, 6, and 7.

#### EXAMPLE II

In another test, a number of 2" diameter carbon plugs were made at 10 and 20 p.p.h. pitch levels from conductive blend charges containing a somewhat coarser petroleum coke flour than that described in Example I. In this series of experiments all of the plugs were initially pressed at temperatures ranging from 700° C. to 900° C. and after removal from the pressure baking mold, were protectively packed in granulated coke flour and rebaked in an electrically heated furnace to 1000° C., to ensure a uniform final temperature, after which the permeability to gas flow of the internal carbon structure of the plug was measured. A set of permeability measurements was made with the direction of gas flow oriented "with" the grain of the carbon structure and another set with the direction of gas flow "against" the grain, i.e. "against" and "with" the direction of application pressure by the molding ram. In the following Table II these measurements are listed opposite sample numbers bearing the subscripts A and W. The table also lists the apparent density and resistivity values obtained as well as the processing conditions.

TABLE II.—GAS PERMEABILITY OF VARIOUS PRESSURE MOLDED CARBON SAMPLES

| Processing, Sample No. | Binder level, p.p.h. | Gas pressure, start-end | Effective mech. press. in mix, p.s.i. | Properties <sup>1</sup> |               |                             |
|------------------------|----------------------|-------------------------|---------------------------------------|-------------------------|---------------|-----------------------------|
|                        |                      |                         |                                       | Density, gm./cc.        | Res., ohm-cm. | Admittance F (ml./sec.-cm.) |
| 1A-----                | 10                   | 0-0                     | 4,200                                 | 1.613                   | .00829        | .1207                       |
| 1W-----                |                      |                         |                                       | 1.597                   | 488           | .1755                       |
| 2A-----                | 10                   | 500-500                 | 4,300                                 | 1.621                   | .00940        | .0907                       |
| 2W-----                |                      |                         |                                       | 1.611                   | 620           | .1866                       |
| 3A-----                | 10                   | 1,000-1,000             | 3,800                                 | 1.611                   | .00870        | .1290                       |
| 3W-----                |                      |                         |                                       | 1.608                   | 652           | .1286                       |
| 4A-----                | 20                   | 500-500                 | 4,700                                 | 1.706                   | .00574        | .0292                       |
| 4W-----                |                      |                         |                                       | 1.702                   | 505           | .0359                       |
| 5A-----                | 20                   | Vacuum 1,300            | 3,900                                 | 1.707                   | -----         | .0300                       |
| 5W-----                |                      |                         |                                       | 1.704                   | .00540        | .0453                       |
| 6A-----                | 20                   | Vacuum 2,500            | 5,200-2,700                           | 1.718                   | .00545        | .0097                       |
| 6W-----                |                      |                         | start-end                             | 1.724                   | 300           | .0139                       |

<sup>1</sup> After rebaking to 1,000° C.

samples were molded from a conductive carbonaceous blend charge of petroleum base calcined coke flour (55 Texas coke flour) and a coal tar pitch binder (175° C.,

It is evident from the data that the admittance of the plugs made from 20 p.p.h. binder mix with pneumatic pressure applied during forming is lower by a factor of

10 to 20 as compared with those made at a lower binder level. In addition to the lower permeability to gas flow the carbon articles have a large increase in apparent density and somewhat lower electrical resistivity.

### EXAMPLE III

In another series of experiments, samples of petroleum coke flour mixes bonded in one case with 105° melting point pitch were heated in a mixer, extruded through a conventional extrusion jumbo into 1" diameter rods, cut into 3" lengths and then pressure baked to about 850° C. in accordance with the process of this invention. In this series of pressure bakes the preformed "green" plugs which were nonconductive were heated by passage of current through the graphite mold liner rather than by direct passage of current as was the case with the articles described in the earlier examples. The extrusion mixes contained petroleum coke 90 flour and pitch proportioned in a weight ratio of 70 parts/30 parts. To this mix 4 parts of petroleum base summer oil was added as an extrusion aid.

After removal from the pressure-bake apparatus the carbon plugs were rebaked conventionally to 1000° C. and then to 3000° C. to convert them to graphite. Plugs which were extruded from these same mixes but not pressure baked were also conventionally baked. A comparison of the apparent density obtained after extrusion and after the 1000° C. and 3000° C. baking step between the pressure-baked and conventionally baked plugs is shown in Table III.

be appreciated that many other forms of comminuted carbon or graphite can be used in the practice of the invention. For example, such materials as pulverized coal, artificial and natural graphites as well as lampblack and gas black in various proportions can be used to impart desired properties in the final carbon or graphite article. In addition, coal tars as well as still higher coking value pitches may be employed as binders. For instance a blend of graphite flour and carbon black bonded with high melting point pitch is found to be particularly effective in obtaining articles having high apparent density.

What is claimed is:

1. In a process for making a formed carbon article from a charge comprising carbonaceous particles and a fusible carbonaceous binder, said binder tending to evolve substances which condense on the apparatus used in said process, said process comprising providing a binder content of greater than about 15% by weight of said carbonaceous charge placing said charge in a mold, subjecting said charge within said mold to a mechanical pressure while simultaneously heating said charge to a carbonization temperature, sealing said apparatus and during the application of said mechanical pressure applying a pneumatic pressure higher than atmospheric pressure from an external source of a non-oxidizing gas to said charge whereby the escape of volatiles from said charge is substantially suppressed and whereby an increase in density and flexural strength is achieved in the formed carbon article.

30 2. The process of claim 1 wherein said pneumatic

TABLE III

| 105° C. M.P. pitch binder, Pressure-Carbonization Conditions <sup>2</sup> |                                    |                     | Green A.D., g./cc. |                  | 1000° C. baked A.D., g./cc. |                  | 3000° C. graph A.D., g./cc. |                  | 800° C. coking value <sup>1</sup> of binder |                                    |
|---------------------------------------------------------------------------|------------------------------------|---------------------|--------------------|------------------|-----------------------------|------------------|-----------------------------|------------------|---------------------------------------------|------------------------------------|
| Initial pressure, p.s.i.g.                                                | Final pneumatic pressure, p.s.i.g. | Approx. temp., ° C. | Control, no press. | Pressure applied | Control, no press.          | Pressure applied | Control, no press.          | Pressure applied | Control, Percent carbon                     | Pneumatic pressure, percent carbon |
| 250                                                                       | 250                                | 800                 | 1.640              | 1.642            | 1.365                       | 1.447            | 1.411                       | 1.514            | 49.9                                        | 71.0                               |
| 500                                                                       | 500                                | 700                 | 1.647              | 1.651            | 1.305                       | 1.495            | 1.411                       | 1.542            | 50.3                                        | 74.3                               |
| 1,000                                                                     | 1,000                              | 800                 | 1.644              | 1.640            | 1.395                       | 1.490            | 1.395                       | 1.534            | 52.3                                        | 77.7                               |
| 2,000                                                                     | 2,000                              | 800                 | 1.659              | 1.654            | 1.353                       | 1.536            | 1.400                       | 1.583            | 57.6                                        | 79.6                               |
| 500                                                                       | 1,400                              | 800                 | 1.650              | 1.655            | 1.348                       | 1.555            | 1.384                       | 1.582            | 58.0                                        | 77.3                               |
| 1,000                                                                     | 2,150                              | 800                 | 1.656              | 1.654            | 1.337                       | 1.552            | 1.426                       | 1.636            | 51.0                                        | 77.2                               |
| <b>150° C. M.P. pitch binder</b>                                          |                                    |                     |                    |                  |                             |                  |                             |                  |                                             |                                    |
| 500                                                                       | 500                                | 800                 | 1.687              | 1.685            | 1.473                       | 1.553            | 1.505                       | 1.604            | 60.7                                        | 80.0                               |
| 1,000                                                                     | 1,000                              | 800                 | 1.658              | 1.666            | 1.420                       | 1.557            | 1.487                       | 1.654            | 61.6                                        | 78.3                               |
| 2,000                                                                     | 2,000                              | 800                 | 1.654              | 1.654            | 1.444                       | 1.623            | 1.532                       | 1.689            | 61.9                                        | 76.9                               |
| 500                                                                       | 750                                | 800                 | 1.690              | 1.686            | 1.435                       | 1.563            | 1.502                       | 1.576            | 58.9                                        | 77.2                               |
| 1,000                                                                     | 2,500                              | 800                 | 1.665              | 1.667            | 1.425                       | 1.642            | 1.498                       | 1.698            | 60.5                                        | 88.2                               |

<sup>1</sup> "Coking value" represents the weight of carbon deposited by the pitch binder at high temperatures relative to the weight of the pitch originally used. <sup>2</sup> Estimated mechanical pressure was approximately 500 lbs./in.<sup>2</sup>

The values shown under the 800° C. Coking value column in the table show the marked increase in percentage of carbon obtained from both kinds of pitch when the plugs were baked under pneumatic pressure.

It should be pointed out that the greater convenience and more rapid processing offered by pre-forming by extrusion would not be possible except for the higher binder levels made usable by the application of pneumatic pressure during the rapid baking step. Low binder levels, not in excess of about 15% by weight of the carbonaceous charge were found to be required for rapid baking prior to the invention. In the above described experiment, charges having a binder level of 30% were successfully processed. Charges containing only 15% binder would not be extrudable. Another advantage for the pre-forming technique is elimination of the need for applying high mechanical pressures to the green carbon during the baking stage. As indicated, the mechanical pressures applied were never more than about 500 lbs./in.<sup>2</sup>.

While all of the examples described were limited to the use of petroleum coke flour-containing mixes it will

50 pressure is between about 20 pounds per square inch and about 2000 pounds per square inch.

3. The process of claim 1 wherein said gas is nitrogen.

### References Cited

UNITED STATES PATENTS

- |           |        |             |       |     |      |
|-----------|--------|-------------|-------|-----|------|
| 3,001,237 | 9/1961 | Balaquer    | ----- | 18  | 54.7 |
| 3,246,056 | 4/1966 | Shea et al. | ----- | 264 | 29   |
| 3,249,964 | 5/1966 | Shaler      | ----- | 18  | 5    |
| 3,336,424 | 8/1967 | Cheney      | ----- | 264 | 89   |

## FOREIGN PATENTS

- 759,160 10/1956 Great Britain.  
876,924 9/1961 Great Britain.

JULIUS FROME Primary Examiner

JOHN H. MILLER, Assistant Examiner

U.S. Cl. X.R.